

1

2,907,683

## FIREPROOFING TEXTILES AND THE LIKE

Raymonde Genevieve Madeline, née Madeline, and Jean François Pathus-Labour, Paris, France, assignors to Firma Deutsche Erdöl A.G., Hamburg, Germany

No Drawing. Application February 8, 1954  
Serial No. 408,998

2 Claims. (Cl. 117—136)

The present invention relates to the fireproofing of textiles and the like materials and to novel fireproofed textile materials.

It is an object of the present invention to provide a process of fireproofing textile materials so as to render the same non-inflammable and incapable of supporting combustion.

It is another object of the present invention to provide novel textile and the like materials such as paper, synthetic fiber materials, and the like impregnated with a novel fireproofing material.

Other objects and advantages of the present invention will be apparent from a further reading of the specification and of the appended claims.

The present invention has as an object thereof a process of treating textile fabrics of all types to hygroscopically condition the fabric in view of impregnating the same so as to render the substances treated according to the process of the present invention inflammable and incapable of supporting combustion and further being able to resist deterioration at high temperatures as well upon contact with flame and gases at high temperature.

It is known that the effect of fireproofing as well as the thermal insulation effect is a function of the coefficient of thermal conduction of the impregnant and of the substance impregnated.

The process of the present invention consists in impregnating the textile fabric of all types of materials such as garments, sacks or other packing materials with an aqueous solution of a derivative of alginic acid. Alginic acid is a high polymer of d-mannuronic acid.

The impregnant is then transferred into an insoluble compound in any convenient manner, for example by treatment with an acid-forming gas.

The precipitated insoluble alginic acid derivative adheres to the textile material and forms an impregnation which because of the properties which will be later described prevents the thus treated textile material from burning.

The water-soluble alginic acid derivative in a solution of which the textile fabric is immersed or otherwise contacted is preferably an alkali metal salt of alginic acid, an ammonium salt of alginic acid, an amine of alginic acid, an ester of alginic acid or an ether of alginic acid. It is further preferred that the aqueous solution contain about 0.5-5%, and preferably 1-2% of the soluble alginic acid derivative.

The precipitation of the insoluble alginic acid derivative is preferably accomplished by treatment with a water-soluble heavy metal salt such as the hygroscopic salt calcium chloride. This heavy metal salt reacts with the soluble alginic acid forming an insoluble heavy metal salt of alginic acid. The useful heavy metal salts are those such as soluble salts of iron, zinc, copper, lead, etc. It is preferable that soluble alkali earth salts such as calcium chloride be used for this purpose and it is further preferable that an excess of calcium chloride be used in precipitating the insoluble derivative of alginic acid.

2

Some of the excess of calcium chloride remains in the textile material after it has been allowed to dry substantially and this calcium chloride due to its hygroscopic properties prevents the material from drying completely.

5 It is another preferred embodiment of the present invention that the insoluble derivative of alginic acid be precipitated by the action of an acid-forming gas or by the action of a solution of an acid. Such acid-forming gases include hydrogen chloride, hydrogen bromide, hydrogen iodide, etc. The term acid-forming gas as used herein refers to those gases which in water solution form acids. Acids which may be used with the present invention include hydrochloric acid, hydrobromic acid, acetic acid, propionic acid, etc.

15 It is still another preferred embodiment of the present invention that either the impregnating solution or the precipitating means contain a water soluble hygroscopic substance such as a polyfunctional alcohol or derivative thereof. This hygroscopic substance is impregnated along with the insoluble alginic acid derivative, into the material and it thereby prevents the material from completely drying out.

The soluble salts of alginic acid include alkali metal salts, ammonium salts, amine salts, etc., i.e. sodium alginic, potassium alginic, ammonium alginic and the like. The soluble ethers and esters of alginic acid include methyl, ethyl, acetyl alginic acid and the like. These derivatives are very similar to salts of alginic acid. However the salts are more preferable with the present invention for reasons of economy.

25 The treatment with the substance which causes formation of an insoluble derivative of alginic acid causes an impregnation into the pores of the material with the insoluble derivative, or a layer is formed over the surface 30 of the material thereby coating the same. The thus treated material is mechanically very strong and is practically impermeable to liquids and gases.

The soluble salts of the heavy metals named above include iron chloride, copper sulfate, lead acetate, etc. 40 These salts may be applied in solid state to the impregnated solution, being therein dissolved by the water of said solution and reacting in said solution with the soluble alginic to form an insoluble heavy metal derivative of alginic acid. It is however preferable to use a solution of such heavy metal salt so as to facilitate this reaction. It is also possible to use water soluble alkali earth salts either in solid form or in solution. These alkali earth salts react with the soluble alginic to form an insoluble alkali earth derivative of alginic acid. The soluble alkali earth salts which may be used include, though 45 are not limited to, calcium chloride, strontium nitrate, barium acetate, etc.

50 The strength of the impregnating layer depends partly on the amount of water given up by the gel through syneresis. The syneresis is to an extent controllable by the concentration, temperature and time of action of the precipitating solution. It is further dependent of course upon the concentration and extent of polymerization of the alginic acid derivative.

To increase the plasticity and elasticity of the impregnation and to prevent this impregnation from completely 55 drying out it is favorable to include a water soluble agent such as glycerine, glycol, glycol ether, etc. in either the impregnated solution or in the precipitating solution.

The exceptional characteristics of the thermal insulation of the insoluble alginic acid derivative with which the material is impregnated according to the present invention will be apparent from the following description, these characteristics allowing for the attainment of the objects of the present invention.

60 70 The attempt to provide fireproof materials have not been very successful and it is known that not only must

the material itself be protected but the objects nearby must also be protected from the flames.

Asbestos cloth has been utilized to provide such protection, but the use of such cloth is both difficult and expensive.

By the present invention, on the other hand, a cloth or fabric is utilized which is treated by immersion in a fireproofing solution. For this purpose one utilizes a material which will serve to support the fireproofing substance, such as jute, paper, threads, synthetic fibers, cotton, and all other substances, of which the web may attain the dimensions of 3 mm. x 3 mm. and wherein the dimensions may vary according to the use to which the material is put.

The impregnation according to the process is made as above described. According to the present invention an agent which has resistance to fire may be included in the impregnation such as a silicious substance, silico-alumina, magnesia-alumina, white clay, asbestos, mica, etc. Preferably, hydrated magnesium silicate is utilized ( $Mg_3(SiO_3)_4 \cdot H_2O$ ). The amount of the fireproofing additive such as hydrated magnesium silicate may vary within relatively wide limits, though preferably the amount is between 0.25-3% by weight.

The essential physical characteristics of the mixture of the alginate and the fireproofing additive are as follows:

The hydrated magnesium silicate is not fusible to straw and its resistance to fire is often utilized, however, the inconvenience of utilizing such substance is that it dries very rapidly and thus loses its properties. This inconvenience is overcome by the combination of the substance with the alginate impregnation of the present invention.

In effect the precipitation reaction, as pointed out above is most favorably attained by means of a hygroscopic salt such as calcium chloride in very concentrated solution. As an example, the impregnation of 1 square meter of a material contains the following:

|                                   |    |
|-----------------------------------|----|
| 20 g. calcium alginate            | 40 |
| 10 g. hydrated magnesium silicate |    |
| 350 g. calcium chloride           |    |
| 1 kg. water                       |    |

It should be noted that the efficacy of the absorption and the desorption of the humidity by the insoluble alginate composition permits the attainment of a great number of applications of the products, for example for special packing purposes.

The impregnations according to the present invention give the materials impregnated therewith the following properties:

(1) Complete impermeability to gas, preventing the access of oxygen of the air to everything contained within the material treated,

(2) The water retained by the hygroscopic properties of the layer of impregnant has a low vapor tension and resists heat for a long time, the absorption of calories by the dehydration and then the evaporation of water assures an efficacious protection of the material,

(3) The impregnated fabric remains resistant to fire even after desiccation and a simple wetting will give the product back all its original characteristics.

It is another embodiment of the present invention to include in the bath in which the insoluble alginate impregnation is produced, antiseptic products such as sodium benzoate, formaldehyde, or phenol derivatives so as to assure preservation.

The following examples are given as illustrative of methods of applying the impregnation and the results of different materials so impregnated.

#### Example I

A sack having large pores i.e. such as those used to transport potatoes, is immersed in a 1.5% aqueous solution of sodium alginate for a few minutes. The thus

treated sack is then further treated with a 40% solution of calcium chloride, i.e. through immersion in such solution, for about 5 minutes. After removing the sack from the calcium chloride solution it is allowed to drain for about an hour so that the major quantity of water is forced out through syneresis. The sack is thus impregnated with a film of calcium alginate which renders the sack fireproof.

#### Example II

A sack made of paper having fine pores is immersed in a 1% solution of sodium alginate to which 5% glycol has been added. This sack is then treated with a solution of hydrochloric acid, likewise containing 5% glycol, for 5 minutes. After a few hours or even after a few days, the sack may be utilized, the impregnating layer remaining elastic even under heat and the sack being substantially fireproof.

#### Example III

Two stacks of straw are laid side by side. A first stack is covered with a sheet of jute impregnated with calcium alginate according to the present invention, and the other stack is covered with a non-impregnated sheet of jute. Both stacks of straw are subjected to an incendiary blast. The second stack of straw burns completely including the sheet of jute covering the same, while the first stack of straw remains protected from the flames and the fire does not spread thereto.

#### Example IV

A stack of straw is completely covered with a textile net impregnated with an insoluble alginate by the process of Examples I or II and is surrounded by stacks of straw which contact the impregnated net covering but which are not themselves covered in the same manner. A fire is started on the non-covered straw. This straw burns completely but the fire does not spread to the covered stack of straw. This stack remains completely protected from the fire.

#### Example V

A fire is started in a field under conditions corresponding to a fire which might start at harvest time. After the fire has extended somewhat in the field, a net impregnated as in Example I or II is spread around the fire. The flames stop at the border of the cloth. After several hours the fire becomes extinguished since it cannot pass further.

#### Example VI

Balls of cotton or artificial textile are enveloped in fabric impregnated with an insoluble alginate and are placed side by side with similar balls prepared according to the usual methods but not covered with a protecting sheet. A fire is started simultaneously about both the covered and the non-covered cotton or synthetic fiber balls. In the non-covered balls the fire rapidly reaches the periphery of the balls and the flames then attack the center. In a short time the cotton balls are completely enveloped by flame. On the other hand the cotton or artificial textile fiber balls covered with the alginate-impregnated textile retain sufficient humidity because of the hygroscopic coating to render combustion extremely difficult and the same do not burn.

#### Example VII

Fires are often started in farms by sparks escaping from electrical agricultural equipment. Therefore to test the present invention there is suspended in a granary a fabric impregnated with an insoluble alginate, the fabric being suspended between the grain and the electrical equipment emitting sparks. This results in a permanent protection and no fire starts even after continued use.

#### Example VIII

Tobacco leaves are rolled into balls of usual dimension

i.e. 1.5 m. high and 2 m. wide and are then enveloped in a cloth impregnated according to the present invention. This tobacco is completely protected from any danger of fire while retaining the humidity in the tobacco.

*Example IX*

Dried fruits are put in a sack impregnated with an insoluble alginate according to the present invention. The humidity of the fruit is retained while protecting the same from danger of fire.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended to be comprehended within the meaning and range of equivalence.

What is claimed as new and desired to be secured by Letters Patent is:

1. A process of fireproofing textile materials, comprising the steps of applying to a textile material an aqueous impregnating solution containing at least one water-soluble compound selected from the group consisting of salts and esters of alginic acid; treating the thus-applied impregnating solution with an excess of hygroscopic calcium chloride so as to precipitate from the thus applied impregnating solution a water insoluble derivative of alginic acid which adheres to said textile material and forms a substantially gas impermeable impregnation preventing said thus impregnated textile material from burning; and allowing the water to drain from the thus impregnated textile material so as to remove the major portion of the water therefrom, said excess of said hygroscopic calcium chloride binding water to said water insoluble alginic acid impregnation and preventing complete drying of the thus impregnated textile material, thereby obtaining an im-

regnated textile material which is substantially gas impermeable and highly resistant to burning and which remains elastic and non-brittle due to said bound water.

2. A process of fireproofing textile materials, comprising the steps of applying to a textile material an aqueous impregnating solution containing water-soluble sodium alginate; treating the thus applied impregnating solution with an excess of hygroscopic calcium chloride so as to precipitate from the thus applied impregnating solution water insoluble calcium alginate which adheres to said textile material and forms a substantially gas impermeable impregnation preventing said thus impregnated textile material from burning; and allowing the water to drain from the thus impregnated textile material so as to remove the major portion of the water therefrom, said excess of said hygroscopic calcium chloride binding water to said water insoluble calcium alginate impregnation and preventing complete drying of the thus impregnated textile material, thereby obtaining an impregnated textile material which is substantially gas impermeable and is highly resistant to burning and which remains elastic and non-brittle due to said bound water.

References Cited in the file of this patent

UNITED STATES PATENTS

|    |           |                 |       |                |
|----|-----------|-----------------|-------|----------------|
| 25 | 1,321,708 | Bradley         | ----- | Nov. 11, 1919  |
|    | 2,387,865 | Van Kleeck      | ----- | Oct. 30, 1945  |
|    | 2,435,701 | Vallandigham    | ----- | Feb. 10, 1948  |
| 30 | 2,436,181 | Rosser          | ----- | Feb. 17, 1948  |
|    | 2,513,416 | Gloahec         | ----- | July 4, 1950   |
|    | 2,568,850 | Fasold et al.   | ----- | Sept. 25, 1951 |
|    | 2,610,957 | Steinman et al. | ----- | Sept. 16, 1952 |

FOREIGN PATENTS

|    |         |               |       |               |
|----|---------|---------------|-------|---------------|
| 35 | 27,606  | Great Britain | ----- | 1898          |
|    | 572,790 | Great Britain | ----- | Nov. 19, 1942 |
|    | 625,609 | Great Britain | ----- | June 30, 1949 |